

**1**

2,923,597

**CREASE RESISTANT CYANOETHYL COTTON  
FABRIC OF RETAINED TENSILE STRENGTH  
PRODUCED BY APPLYING A METHYLOL  
MELAMINE RESIN**

Theodore F. Cooke, Martinsville, N.J., John W. Eastes, Ridley Park, Pa., and Linton A. Fluck, Basking Ridge, N.J., assignors to American Cyanamid Company, New York, N.Y., a corporation of Maine

No Drawing. Application March 31, 1955  
Serial No. 498,453

**1 Claim. (Cl. 8—129)**

This invention relates to an improved wrinkle and crease resistant fabric from cyanoethylated cotton.

There is a demand for wrinkle and crease resistant cotton fabrics for example women's dressgoods and the like. In the past this has been effected by treating the fabric with a thermosetting resin such as melamine formaldehyde, urea formaldehyde and ethylene urea formaldehyde and the like. The desirable property of wrinkle and crease resistance has been obtained at the expense of serious disadvantage, namely marked loss in tensile and tear strength. It is a generally accepted theory that the crease and wrinkle resistance results from a chemical reaction of the resin with the hydroxyl groups of the cellulose molecule so that the long chains of cellulose are cross linked at suitable intervals by a resin bridge, resulting in the increase in wrinkle resistance but also decreasing the extensibility so that under stress the fabric breaks or tears at a much lower degree of force than is the case with the original cotton which has greater extensibility. In the past the serious disadvantage of lowered tensile strength and poor tear resistance has been endured in order to obtain the advantages of crease and wrinkle resistance, but the field of utility of crease and wrinkle proofed fabric has been seriously reduced because in cases where the fabric needs high degree of tensile strength or tear resistance, the treated fabric is unsuitable.

According to the present invention it has been found that cyanoethylated cotton which is a recent development and in which the cotton is reacted with acrylonitrile and caustic alkali so that a portion of the hydroxyl groups are transformed into beta-cyanoethoxy groups can be treated with thermosetting resins in exactly the same manner as cotton fabrics but the resulting fabric although having the same degree of high wrinkle and crease resistance has the advantage of being almost as strong, in some cases actually as strong, as untreated cyanoethylated fabric and shows a markedly improved tear resistance.

It is not known why the cyanoethylated cotton after resin treatment should show such remarkable increase in tensile and tear strength over ordinary resin treated cotton fabric. In fact, as far as the accepted theory is concerned, it is quite incomprehensible because the cyanoethylated cotton which is useful, that is to say, cotton which still retains its cotton structure normally has less than a third of its hydroxyl groups changed into beta-cyanoethoxy groups. The best cyanoethylated cotton

**2**

ranges from 3.5—5.5% nitrogen, although material as low as around from 3% nitrogen is still useful, and higher degrees of cyanoethylation up to the point where one of the three hydroxyl groups on the anhydroglucoside unit of the cellulose has reacted can also be employed. In other words, there is an enormous excess of remaining free hydroxyl groups over that required to react with the small amount of resin which is used in crease proofing so that chemically there is no reason why the cross linking should not be as full and as extensive with cyanoethylated cotton as with cotton itself. In fact, as far as the wrinkle and crease resistance is concerned, this appears to be borne out because the two products are substantially the same in this respect. It is not known why there is such a marked reduction in tensile strength loss and it is not desired to limit the present invention to any theory of action which would explain the retention of the wrinkle and crease resistance without the great loss in tensile strength.

20 A further advantage of the present invention lies in the fact that the resin treated cyanoethylated cotton has all of the desirable characteristics of cyanoethylated cotton such as high degree of resistance to mildew and similar micro-organisms, increased heat resistance and the like.

25 Another advantage of the present invention is that the resin treatment is not changed and the same conventional methods may be used with cyanoethylated cotton. No new application technique therefore needs to be learned.

The invention will be described in greater detail in 30 conjunction with the following examples in which the parts are by weight unless otherwise specified.

**EXAMPLE 1**

A piece of 80 x 80 bleached unmercerized cotton print 35 cloth is treated with acrylonitrile to give a nitrogen content of about 3.4%. The cyanoethylated product is then treated with the following composition:

7.5 parts trimethyl trimethylol melamine. (This is resin No. 1.)  
0.9 part urea  
0.4 part mixed isopropanolamine hydrochloride  
91.7 parts water

The fabric is passed through this composition and then 45 through a three bowl mangle with two dips and two nips to give a pick-up of about 80% of the liquid composition after which it is dried at about 225° F. and then subjected to a heat treatment at 350° F. for about one minute.

50 A second piece of the 80 x 80 bleached unmercerized cotton print cloth but which has not been cyanoethylated is then treated in the same solution as above by the same procedure. This is used as a control.

The cyanoethylated fabric on soil burial in a standard 55 virulent soil showed no attack after two weeks, whereas untreated cotton cloth is substantially disintegrated.

An examination of the resin treated cotton and cyanoethylated cotton fabrics showed that the cyanoethylated cotton possessed a superior luster.

60 Pieces of each of the above-treated fabrics are then tested for wrinkle resistance by the method 14—53 described on page 154 of the 1954 edition of the Technical

Manual and Year Book of the American Association of Textile Chemists and Colorists and the results follow:

| Treatment                                              | Wrinkle Resistance, degrees | Total Tensile Strength, lbs. |
|--------------------------------------------------------|-----------------------------|------------------------------|
| Untreated 80 x 80 cotton print cloth                   | 140                         | 107                          |
| Untreated 80 x 80 cotton print cloth +7.5% Resin No. 1 | 197                         | 85                           |
| Cyanoethylated 80 x 80 cloth                           | 138                         | 101                          |
| Cyanoethylated 80 x 80 cloth +7.5% Resin No. 1         | 177                         | 100                          |

## EXAMPLE 2

The procedure of Example 1 is repeated using, however, 10 parts of Resin No. 1 and the treated fabric is

5 The procedure of Example 1 is followed replacing the methylated trimethylol melamine resin with 3.4% of a reaction product of methylol stearamide and methylated trimethylol melamine plus 13.5% of urea formaldehyde, the catalyst being replaced by ammonium sulfate.

4 EXAMPLE 4

The procedure of Example 1 is followed replacing the methylated trimethylol melamine resin with 3.4% of a reaction product of methylol stearamide and methylated trimethylol melamine plus 13.5% of urea formaldehyde, the catalyst being replaced by ammonium sulfate.

## EXAMPLE 5

10 The procedure of Example 1 is repeated replacing the isopropanol amine hydrochloride with magnesium chloride, the amounts of solids are 5.4% instead of 7%.

## EXAMPLE 6

15 The treated products of Examples 4 and 5 were then tested and the results follow:

## Wrinkle recovery

| Treatment                       | Initial |      | Total | After 1 Sanf. Wash |      | Total | Tensile Strength |      | Elmendorf Tear Strength |      |  |  |
|---------------------------------|---------|------|-------|--------------------|------|-------|------------------|------|-------------------------|------|--|--|
|                                 | Warp    | Fill |       | Warp               | Fill |       | Warp             | Fill | Warp                    | Fill |  |  |
|                                 |         |      |       |                    |      |       |                  |      |                         |      |  |  |
| Example 4:<br>80 x 80 Cotton    | 125     | 130  | 255   | 86                 | 87   | 173   | 40               | 26   | 1.28                    | 0.75 |  |  |
| Cyanoethylated Cotton           | 116     | 115  | 231   | 92                 | 98   | 190   | 52               | 38   | 1.60                    | 0.35 |  |  |
| Example 5:<br>80 x 80 Cotton    | 114     | 114  | 228   | 97                 | 106  | 203   | 39               | 29   | 1.13                    | 0.58 |  |  |
| Cyanoethylated Cotton           | 120     | 126  | 246   | 110                | 110  | 220   | 54               | 29   | 1.25                    | 0.68 |  |  |
| Untreated Cotton                |         |      |       |                    |      |       | 53               | 41   | 1.62                    | 1.18 |  |  |
| Untreated Cyanoethylated Cotton |         |      |       |                    |      |       | 63               | 43   | 1.73                    | 1.35 |  |  |

dried at a low temperature and then subjected to a heat treatment as in the preceding example.

They are then tested for wrinkle resistance and tensile strength as in the preceding example and the results follow:

| Treatment                                           | Wrinkle Resistance, degrees | Total Tensile Strength, lbs. |
|-----------------------------------------------------|-----------------------------|------------------------------|
| Untreated 80 x 80 cotton cloth                      | 140                         | 110                          |
| Untreated 80 x 80 cotton cloth plus 10% Resin No. 1 | 258                         | 53                           |
| Cyanoethylated 80 x 80 cloth                        | 138                         | 116                          |
| Cyanoethylated 80 x 80 cloth plus 10% Resin No. 1   | 255                         | 83                           |

## We claim:

A wrinkle-resistant, crease-resistant, partially-cyanoethylated cotton fabric containing cyanoethyl groups in an amount not exceeding one such group per anhydroglucose unit thereof, the cotton fibers containing from 3.5 to 5.5% by weight of nitrogen in the form of cyano groups, prepared by applying to said cyanoethylated cotton fabric an aqueous dispersion of about 7.5% by weight of trimethyl trimethylol melamine and a catalyst, drying 35 the so-treated fabric and heating the dried fabric at curing temperatures until the trimethyl trimethylol melamine is transformed into a thermoset, insoluble product firmly attached to the surface of said fibers.

40 45 References Cited in the file of this patent

UNITED STATES PATENTS

2,373,136 Hoover \_\_\_\_\_ Apr. 10, 1945  
 2,375,847 Houtz \_\_\_\_\_ May 15, 1945  
 2,423,428 Pollard \_\_\_\_\_ July 1, 1947  
 2,473,308 Stallings \_\_\_\_\_ June 14, 1949  
 2,715,078 Cohen \_\_\_\_\_ Aug. 9, 1955

## OTHER REFERENCES

55 Amer. Dyestuff Reporter, November 22, 1954, pp. P774-P779.  
 Compton: Textile Res. Jour., January 1955, pp. 58 and 68-72.  
 Daul: Textile Res. Jour., March 1955, pp. 246-253.

## EXAMPLE 3

The procedure of Example 1 is repeated using 10 parts of dimethylol ethylene urea resin (Resin No. 2) instead of the methylated trimethylol melamine resin.

They were then tested as in Example 2 and the results follow:

| Treatment                                                | Wrinkle Resistance, degrees | Total Tensile Strength, lbs. |
|----------------------------------------------------------|-----------------------------|------------------------------|
| Untreated 80 x 80 cotton cloth                           | 140                         | 110                          |
| Untreated 80 x 80 cotton cloth plus 10% Resin No. 2      | 251                         | 51                           |
| Cyanoethylated 80 x 80 cotton cloth                      | 138                         | 116                          |
| Cyanoethylated 80 x 80 cotton cloth plus 10% Resin No. 2 | 251                         | 82                           |